

Feb. 3, 1931.

L. D. GRISBAUM

1,791,473

OIL RECLAMATION

Filed Aug. 4, 1927 6 Sheets-Sheet 1



Inventor:  
Leonard D. Grisbaum  
By his Attorneys  
Symmetswelt + Lechner

Feb. 3, 1931.

L. D. GRISBAUM

1,791,473

OIL RECLAMATION

Filed Aug. 4, 1927

6 Sheets-Sheet 2

Fig. 1b



Inventor

Leonard D. Grisbaum  
By his Attorneys  
Symmetzelt & Lechner

Feb. 3, 1931.

L. D. GRISBAUM

1,791,473

## OIL RECLAMATION

Filed Aug. 4, 1927

6 Sheets-Sheet 3

Fig: 2<sup>a</sup>



Feb. 3, 1931.

L. D. GRISBAUM

1,791,473

OIL RECLAMATION

Filed Aug. 4, 1927

6 Sheets-Sheet 4

Fig: 2<sup>b</sup>.



Inventor  
Leonard D. Grisbaum  
By his Attorneys  
Synnestvedt & Lechner

Feb. 3, 1931.

L. D. GRISBAUM

1,791,473

OIL RECLAMATION

Filed Aug. 4, 1927 6 Sheets-Sheet 5



Feb. 3, 1931.

L. D. GRISBAUM

1,791,473

OIL RECLAMATION

Filed Aug. 4, 1927 6 Sheets-Sheet 6



INVENTOR  
Leonard D. Grisbaum  
BY  
Symmetweld & Lechner  
ATTORNEYS

## UNITED STATES PATENT OFFICE

LEONARD D. GRISBAUM, OF INDIANAPOLIS, INDIANA, ASSIGNOR TO RAILWAY SERVICE & SUPPLY CORPORATION, OF INDIANAPOLIS, INDIANA, A CORPORATION OF INDIANA

## OIL RECLAMATION

Application filed August 4, 1927. Serial No. 210,545.

This invention relates to the reclamation of oils, particularly mineral lubricating oils which have been used with fibrous waste material such as is commonly used in the lubrication of railway journals.

My process is particularly adapted to treat and renovate lubricating oils of the above character which are normally unfit for further service. Such oils constitute a liquid of a black viscous nature in some degree of emulsion and may contain reclaimable oil, water, colloidal dirt, heavy extraneous solids, such as particles of metal and silicates, finely divided fibrous material or lint, and dye stuffs from the fibrous material. Any one or all of these foreign substances may have been entrained and/or absorbed by the oil according to the class of service in which the oil was used. The oil may also contain some metallic soap such, for example, as lead oleate. Such metallic soaps are often placed in mineral oils during their preparation for lubricating purposes and their presence in the oil is considered to be advantageous for certain classes of service. However, in many instances, it has been found that it is desirable that the oil should be free of such metallic soaps.

It is the primary object of the present invention to recondition such oil by removing not only all the dirt and foreign substances from the oil, but also any metallic soap which may be present. I accomplish the foregoing by chemically and mechanically treating the oil as will be fully set forth below.

Other objects and advantages incident to my invention will appear to those skilled in the art from a consideration of the following description and the appended drawings which illustrate the preferred embodiment of the apparatus for carrying out the method.

## Of the drawings—

Figs. 1a and 1b placed together at their lines X—X form a somewhat diagrammatic plan view of a suitable layout of the apparatus; and

Figs. 2a and 2b placed together at their lines Y—Y form a somewhat diagrammatic side elevation of the layout of Fig. 1.

Figs. 3a and 3b placed together at their

lines Z—Z form an end view taken from the right of Fig. 2.

Certain parts and connections are omitted from the various figures in order to reduce unnecessary complication.

Referring now to the drawings, it will be seen that the apparatus comprises a number of tanks marked A, B, C, D, E and F which may be supported on any suitable structural work. It will be observed that two tanks C identical in construction are shown.

Tank A is the treating-chemical mixing tank. It is supplied with water from the cold water supply connection 4 through the valved connection 5 and may be drained through the outlet 6 communicating with any suitable sewage line 7. The mixed chemicals are passed into a treating tank C through connections 8 by any suitable pump 9 which has an intake 10 terminating in the bottom of the tank A. Valves 11 control the flow through the connections 8 through the inlets 12 to the treating tanks C.

The water heating tank B is supplied from the connection 4 through the piping 13. This tank is provided with a vent 14 to the atmosphere. The water may be heated in this tank in any suitable manner as by a series of steam coils (not shown).

As the tanks C are identical in construction, the description of them will refer to one of them only.

Tank C is provided with a conical bottom 15. The inlet 12 enters the tank at the apex of its conical bottom. A jacket 16 surrounds this tank and has a bottom 17 conically shaped to correspond with the cone 15. An opening 97 is provided in the top of the tank C.

Adjacent the top of tank C are a number of spray nozzles 18 which are provided with a connection 19 and a valve 20 for admitting hot water through the piping 21 which communicates with the bottom of tank B.

Water is supplied to the jacket 16 from the piping 21 through valved connection 22 and may be drained therefrom to the sewer 7 through the valved pipe 23 and pipe 24. A steam heating coil 25 is positioned within the jacket 16 and is provided with a valved inlet 100

26 and a trapped drain 27. The inlet 26 receives steam through the steam supply connections 28.

An air jet 29 terminates inside the tank C just above the inlet 12. A valved connection 30 supplies the jet 29 with air under pressure from the supply pipe 31. An oil drain 32, pivoted at 33, communicates with the outlet piping 34. Any suitable means, such as the chain 35, may be provided for regulating the level of the oil drain 32.

The oil to be reclaimed is pumped into a tank C through the pipes 39, 8 and 12.

The tank C may be drained through the pipe 24.

The piping 34 terminates inside the perforated bell 36 positioned in the bottom of tank D. Water may be admitted to this tank through the valved connections 37 and may be drained therefrom through the valved drain 38.

Horizontally disposed within tank D are a number of perforated baffles 40 and at the top of this tank is a more or less conically shaped hollow heating plate 41. Steam is supplied to the interior of the plate 41 through the valved connection 42 which communicates with the steam supply pipe 28 and is exhausted therefrom through the trapped pipe 43 which connects with the drain 38. A collecting cone 44 is positioned above the heating plate 41 and the collecting cone and the plate are each provided with an oil overflow opening 45 and 46, respectively, which are located at their highest points.

At one side of the collecting cone 44 is a spillway which is adapted to deliver the oil to the color meter 47. A communication 48 and valve 49 serve to carry the oil from the meter 47 to the dehydrating tank E.

The tank E is made conical at top and bottom and the inlet 50, communicating with the pipe 48, enters the tank at the apex of the bottom cone. This tank is provided with a steam jacket 51 which covers its entire outer surface.

The jacket 51 is provided with a valved steam supply connection 52 communicating with the supply pipe 28 and a trapped drain 53 which discharges into the sewer through 54 and 55.

A valve 98 is provided for breaking the seal after the dehydrating operation.

A pipe 55 communicates with the apex of the top cone of tank E and with the condenser 57. This condenser is provided with tube sheets 58 and 59 between which tubes 60 extend. A vertical baffle 61 divides the chamber formed in the condenser above the sheet 58. Pipe 56 enters one of the chambers above the sheet 58. A vacuum pump 62, driven by a suitable motor 63, is provided with a connection 64 to the other one of the chambers above the sheet 58.

The space around the tubes 60 between the sheets 58 and 59 is supplied with cold water

through connections 65 which connect with the cold water line 37. This space drains through pipes 66, 54 and 55.

The sump in the condenser below the sheet 59 may be drained through the valved pipe 67.

A connection 68 and valve 69 are provided for passing the oil from the tank E to any suitable storage tank 70.

A pump 71 driven by the motor 72 is provided with an intake line 73 extending into the storage tank 70. This pump is adapted to deliver the oil to any point of use or to other storage tanks through the valved connections 74 and 75, respectively. By manipulation of the valves 76 in line 73, and the valves 77, 78 and 79, the pump may be used for pumping oil from the storage tank or tanks, to which the line 75 leads, to any point of use.

The sludge treating or process tank F is identical in construction with the tanks C. Its jacket 16 and nozzles 18 are supplied with hot water from tank B through the pipes 21 and 80, and its air jet 30 from the compressed air supply 31 through the valved connection 81. Steam is supplied to its heating coil 25 through the valved pipe 82 and the supply line 28 and is exhausted therefrom through the trapped drain 83 and pipe 84. Water may be drained from the jacket 16 through the outlet 85 and pipe 84.

A connection 86 communicates, at one end, with the piping 8 through valve 87 and at its other end with the bottom of the tank F through pipe 88, valve 90 and pipe 89. A valved communication 91 connects the outlet pipes 34 of tank C with the pipe 88. Tank F may be drained through pipe 89 and valved connection 92.

The outlet 32 of tank F communicates with the intake 93 of pump 94 which is driven by motor 95. This pump is adapted to deliver oil from tank F, through piping 96 and 34, to tank D.

The tanks B, C, E and F are all provided with heat retaining lagging 99.

In order to recondition oil of the character hereinbefore outlined, I treat the oil to counteract its colloidal condition and break its emulsion, to decompose organic matter entrained from the waste with which it has been used, to neutralize any acids present and to render basic any metallic soaps which may be present. I accomplish these various steps by the use of some alkaline chemical, such, for example, as caustic soda (NaOH) or caustic potash (KOH). I prefer to use what is known in the art as a strong-base caustic as distinguished from what is known as weak base caustics and in carrying out my process I use 76% commercial caustic soda of the flake variety, its characteristics being better adapted for handling, as it is readily soluble and practically dustless.

In carrying out the method by the apparatus shown a quantity of caustic soda is measured out by weight and placed into the tank A. Water is admitted to tank A from the supply pipe 5 and the chemical is dissolved therein. This solution is then pumped into one of the tanks C through line 8. The dirty oil is now pumped into the tank C through connections 39 and 8, carrying with it all the solution remaining in line 8. The oil passes upwardly through the solution in this tank and thoroughly mixes therewith.

I have found that, in order to effectively accomplish all the steps outlined above, which steps are necessary for complete reconditioning and to accomplish them without producing objectionable reactions, it is highly desirable that the quantity of treating chemical should be from 3 to 6% (say 5%) by weight of the oil to be treated. I prefer also to dissolve the chemical in water to form a 20 to 25% solution, (say 25% chemical and 75% water by weight). For example: A tank C is adapted to treat a batch of oil weighing about 4000 pounds. This would require a solution of 200 pounds of dry chemical and 600 pounds of water. It is to be understood that the quantities, given above, apply when using 76% commercial caustic soda which I prefer. They would vary, of course, with other chemicals which might be used.

It is a well known fact that oil has a relatively high coefficient of expansion, and, as the oil is measured into the tank C by volume, it is necessary that it should always enter at, or approximately at, the same temperature in order to insure uniform batches by weight.

As the chemical is dissolved in the water, the temperature of the resultant solution rises, and I prefer to use the solution in its hot state (about 170°-200° F.). I prefer also to admit the oil at approximately the same temperature (170°-200° F.). This temperature is only slightly below the treating temperature maintained in the treating tank, and, therefore, I am enabled to reduce the time of treatment of a batch as it is not necessary to raise the temperature of the mixture more than a few degrees to reach treating temperatures.

The temperature of the mixture is raised to and maintained at a point slightly above the boiling point of water, say, 215°-220° F. This is effected by partially filling the jacket 16 (to about the level indicated by the line L in Fig. 2<sup>a</sup>) sealing the jacket (by closing the valves in its supply and drain lines 22 and 23, respectively) and passing steam at about 15 pounds pressure through the heating coil 25.

The mixture is maintained at this temperature for a period of about two hours and during this time it is subjected to violent agitation of about one minute duration at five minute intervals. These agitations are effect-

ed preferably by means of the air jet 29 which terminates in the apex of the cone at the bottom of the tank. This position of the jet insures a very thorough agitation throughout the entire mass as the agitation is initiated at its lowest point and moves upwardly.

All the chemical reactions take place during this period of agitation. The colloidal condition of the oil is counteracted, offering the demulsifying reagent more ready access to every part of the oil. Any acids present are neutralized and a large percentage of organic matter is decomposed.

It should be noted here that air agitations are preferred because they are the most effective for driving off the gases formed by the decomposition of the organic matter. If some mechanical stirring means was used for agitating the mass, these gases could only escape very slowly and would greatly retard the subsidence of the mixture which follows the treating or processing period.

The organic matter (including short ends and lint picked up from the fibers of the packing with which the oil is used) should be removed because its presence may interfere with the proper lubrication of the journal. Small fibrous pieces of this nature are not long enough to aid in transferring lubricant from the reservoir at the bottom of the box to the surface of the journal, and, furthermore, they have a tendency to collect in sort of matted masses, either at the surface of the bearing itself, or in corners of a box adjacent thereto, in such manner as to impair or retard the flow of the oil. Such mats of fibrous material frequently ignite as the result of the heat generated by the poor lubrication and a hot box develops. It is also my opinion that the presence of organic matter of this kind is largely responsible for the extremely tenacious character of the emulsion existing in used journal box oils, and by removing it in the manner accomplished by the present invention, I greatly facilitate the breaking down of the colloidal and emulsified condition of the oil.

I have found that periodic agitations are much more effective for aiding and augmenting the reaction of the chemical and any metallic soap which may be present to render the soap basic, than one continuous agitation equal to or greater than the sum of the intermittent agitations. This may be due to the fact that the chemical undoubtedly takes a shorter period of time (say about 5 minutes) to react with the soap, and then that chemical, which has been immediately adjacent the soap, may become used up, so to speak. In which case the succeeding agitation would undoubtedly bring fresh chemical in contact with the soap. Or it may be that the agitations bring unreacted parts of

the soap in contact with the chemical; or both.

In rendering the soap basic, it becomes insoluble in the oil and is taken over into the chemical solution.

One of the most common of metallic soaps which are placed in lubricating oils, is lead oleate, the formula for which is



10 By rendering such a soap basic by this process, the soap probably takes on two hydroxides from the treating solution. This would result in the formula  $(C_{18}H_{38}O_2)_2Pb(OH)_2$ , which represents a basic lead soap. Such a basic soap is insoluble in petroleum, and, hence, is taken over into the treating solution.

15 After the approximate two-hour period of agitation in the tank C all the foreign substances have been liberated from the oil and are held in suspension in the mixture. If the mixture were allowed to subside and cool, all the extraneous matter would settle to the bottom of the tank but this would require a relatively long period of time, as the mass is relatively dense and viscous. In order to cause a separation and subsidence in the least possible time, I reduce the viscosity of the 20 mass by spraying it with water, preferably at a temperature slightly below that of the treated mixture, say 200° F. The amount of water thus added should be about 25%, by volume, of the entire mass.

25 The mass is now subjected to a final agitation, lasting for a period of about five minutes and then the heating is stopped. The water reduces the viscosity of the mass as a whole and absorbs caustic soda from the treating solution, for which it has a strong affinity. The mixture, being relatively fluid on account of its temperature and having a relatively low viscosity in view of the added 30 water, subsides very rapidly.

35 The fact that the top part of the tank is unjacketed and unlagged and that the jacket is not entirely filled with water assists in promoting a very rapid settlement as the upper layer of the oil in the tank will cool more rapidly than the mass as a whole. This 40 layer is more viscous and tends to increase the surface tension of the mixture and thereby reduce bubbling and agitation at the surface with the result that subsidence and separation are further expedited.

45 The heavy extraneous solids subside to the bottom of the tank, the treating fluid, containing dye stuffs and the lead soap, settles above the heavy matter at the bottom and the 50 oil rises to the top above the treating solution.

55 It is to be noted that all the treating steps are carried on at atmospheric pressures as the opening 97 of tank C always remains un- 60 covered.

After subsidence of the mixture in tank C the clean oil may be drawn off thru the outlet 32 and pipes 34 to the separating tank D. The oil passes upwardly through this tank and in its progress is broken up into fine streams by the perforated baffles 40. This action helps to remove particles of water which may be entrained in the oil. Such droplets or particles subside to the bottom of the tank from where they may be removed thru the drain line 38. As the oil rises in the tank D, toward and thru the outlet 46 it contacts with both sides of the hollow heating plate 41. This action also aids in removing entrained water from the oil as the water contacting with the plate, which is heated to about 230° or 240° F., vaporizes and escapes upwardly thru the opening 45 in the collecting cone 44.

70 The collecting cone is set slightly off the horizontal and the oil collects at its low side, from where it flows over the meter 47 for inspection to the dehydrating tank E.

75 Under certain conditions it may be found that the oil still contains a perceptible quantity of treating chemical when it leaves the treating tank C to enter the tank D. This chemical may be removed by admitting a substantial quantity of water into the tank D, say to about three quarters full. The oil in passing upwardly thru the water is broken up into fine streams and is scoured, so to speak, by the water. The heating plate 41 of course operates, as before, to drive off entrained water.

80 In the tank E the oil is subjected to the final drying operation. This operation is particularly adapted to remove what might be termed "moisture" in the oil, in contradistinction to "entrained water" or to oil in an "emulsified" condition. The oil enters this tank thru the inlet 50 and a normal charge would fill the tank to about the bottom of the top cone. The vacuum pump 62 is now started and steam, at about 15 pounds pressure, circulated thru the jacket 51. Any moisture still remaining in the oil is driven off and is drawn out of the tank E into the condenser tubes 60 where it condenses and collects in the sump below the sheet 59. Condensate may be removed from the sump by 85 opening the valve in the drain 67.

85 In view of the fact that cold water is circulated around the tubes 60 I am enabled to carry relatively high temperatures in the tank E without overheating the vacuum pump by the vapor drawn thru the condenser, as substantially all the moisture will condense in the tubes 60 and drop into the sump. The vacuum pump is adapted to reduce the pressure on the surface of the oil to about that pressure which would correspond to from 20 to 25 inches of mercury and hence the moisture will be driven off very rapidly, especially since the oil is heated to 90

a temperature of about 240° F., or that which corresponds to steam at about 15 pounds pressure.

It is to be noted in connection with the construction of tank E that its conical top and bottom provides for additional heating area and greater strength and also provides a point of concentration for the vapor drawn off thru the pipe 56 as well as a low point 10 from which the tank may be drained. It is further to be noted that the jacket surrounding this tank covers its entire outer surface including the conical portion above a normal charge of oil. It is so constructed 15 in order to prevent the vapor rising from the oil from condensing and falling back into the body of oil, as would occur if this vapor rose and contacted with an unjacketed portion of the wall.

20 After a sufficient period of time has elapsed for complete dehydration of the oil, the vacuum pump is stopped, the steam to the jacket is shut off, and the seal of the tank is broken (by means of the valve 98). The 25 completely reconditioned oil may now be passed into the storage tank 70 thru the connection 68.

The oil may be delivered from the storage tank 70 to any other suitable storage tank 30 thru connections 73, pump 71 and pipes 74 and 75, and may be pumped from there, or from the tank 70 (thru the line 74) by the same pump to any suitable place of use, such, for example, as an adjacent plant for 35 waste impregnation.

After the oil has been drawn off from the treating tank C the treating solution and sludge still remain at the bottom. This mass 40 contains a certain quantity of reclaimable oil. In order to obtain this oil I agitate the solution and sludge, and thereby place the sludge in suspension in the solution, and drain the mass into the sludge treating tank F thru the outlet 32, pipes 34, 91, 88 and 89. 45 This will transfer all the mass from tank C to tank F except a small quantity of the relatively heavy solids which will quickly settle in the cone at the bottom of the tank below the lowest point which the outlet 32 is adapted to drain. This very heavy matter 50 may be drained to the sewer thru the pipe 24.

If desired all of the mass remaining in the tank C after a treating operation, including the heavy solids, may be passed into tank F thru the pipes 23, 8, 86, 88 and 89.

The sludge now in tank F is allowed to settle for a period of about 10 or 12 hours after which time the remaining oil will be 60 found at the top of the mass, the treating solution will be found below the oil and the relatively heavy sludge particles will be found at the bottom. The oil may now be drained from the top thru the outlet 32 of the tank F and passed (by means of the pump 94) thru the pipes 93, 96 and 34 into the sepa-

rating tank D. Its treatment from this point on is identical with the treatment of the oil passed directly into tank D from tank C. The treating solution may now be drained from the tank F for reuse.

If the treating solution has been used sufficiently to exhaust its power to act as a counter-colloidal and a demulsifying reagent, or if it has absorbed lead soap to a point approaching saturation, it is passed off to any suitable point where the lead soap may be precipitated out of it in the form of a lead salt which may be used commercially in a number of ways. This can be accomplished in any suitable manner, as by treating the solution with nitric or sulphuric acid.

Any residual sludge remaining in tank F, after removal of the oil and the solution, may be drained to the sewer thru pipes 89 and 84.

If desired the tank F may be used in the same manner as tanks C. In other words, as a primary treating tank, for which purpose it has been constructed exactly the same as tanks C. If it is so used, the treating chemical and dirty oil are pumped into it thru the lines 8 and 86.

The use to which tank F is put depends upon the type and condition of the oil being treated.

It will be noted that, as far as possible, the various tanks of the plant are mounted at relative levels such that the oil may be passed from one tank to another in the process without the necessity of pumping.

According to the above process I am able to reclaim practically all of the oil, by volume, contained in the viscous and emulsified mass delivered to the plant. As an example, one gallon of dirty oil at about atmospheric temperatures weighs about 8 pounds. As it is delivered from the plant, its volume is practically identical (at the same temperature) but it weighs only about 7½ pounds. The one half pound difference represents, of course, all the extraneous matter and heavy solids which have been removed.

In many cases the oil as delivered from the plant is more suitable for use as a lubricant than the same oil was when it was originally put into service. Its viscosity is higher than many new and unused lubricating oils. Thus, it is often advantageous to treat commercial lubricating oil according to my new process before the oil is even placed in service, not only to remove undesirable metallic soaps but also to improve its lubricating qualities.

Attention is called to the fact that certain of the subject matter disclosed and claimed herein is also disclosed in my copending application Serial No. 74,949, filed December 12th, 1925, the claims of said copending application, however, being limited to other features.

I claim:—

1. A lint free reclaimed journal box lubricating oil.
2. Apparatus for reclaiming used journal box lubricating oil including in combination, a tank adapted to receive a charge of oil to be reclaimed, and means for heating the charge in the tank including a jacket surrounding the lower portion of the tank and terminating substantially below the point to which the tank is adapted to be charged, means for admitting water to the jacket and means for heating the water.
3. Apparatus for reclaiming used journal box lubricating oil including in combination, a tank adapted to receive a charge of oil to be reclaimed, and means for heating the charge in the tank including a jacket surrounding the lower portion of the tank and terminating substantially below the point to which the tank is adapted to be charged, means for admitting water to the jacket and means for heating the water, together with means for sealing the jacket.
4. Apparatus for reclaiming used journal box lubricating oil including in combination, a tank adapted to receive a charge of oil to be reclaimed, and means for heating the charge in the tank including a jacket surrounding the lower portion of the tank and partially filled with water so that the level of the water is below the point to which the tank is adapted to be charged, and means for heating the water, the jacket being adapted to be sealed.
5. The method of renovating contaminated, emulsified, car journal, lubricating oil which has been used with waste, which includes treating the oil by mixing therewith an alkaline solution of sufficient strength to break the emulsion and react with contaminations including lint, the treatment being conducted at a temperature above approximately 170° F. and preferably in the neighborhood of the boiling point of water, adding water to the mixture and then removing supernatant oil after subsidence of the mixture.
6. The method of renovating contaminated, emulsified, car journal, lubricating oil which has been used with waste, which includes treating the oil by mixing therewith an alkaline solution of sufficient strength to break the emulsion and react with contaminations including lint, the treatment being conducted at a temperature above approximately 170° F. and preferably in the neighborhood of the boiling point of water, adding water to the mixture, agitating the mixture, and then removing supernatant oil after subsidence of the mixture.
7. The method of renovating contaminated, emulsified, car journal, lubricating oil which has been used with waste, which includes treating the oil by mixing therewith an alkaline solution of sufficient strength to break the emulsion and react with contaminations including lint, the treatment being conducted at a temperature above approximately 170° F. and preferably in the neighborhood of the boiling point of water, agitating the mixture, and separating renovated oil from the mixture.
8. The method of renovating contaminated, emulsified, car journal, lubricating oil which has been used with waste, which includes treating the oil by mixing therewith an alkaline solution of sufficient strength to break the emulsion and react with contaminations including lint, the treatment being conducted at a temperature above approximately 170° F. and preferably in the neighborhood of the boiling point of water, agitating the mixture, mixing water therewith, and separating renovated oil from the mixture.
9. The method of renovating contaminated, emulsified, car journal, lubricating oil which has been used with waste, which includes treating the oil by mixing therewith an alkaline solution of sufficient strength to break the emulsion and react with contaminations including lint, the treatment being conducted at a temperature above approximately 170° F. and preferably in the neighborhood of the boiling point of water, adding water to the mixture, agitating the mixture, and then separating renovated oil from the mixture.
10. The method of renovating contaminated, emulsified, car journal, lubricating oil which has been used with waste, which includes treating the oil by mixing therewith an alkaline solution of sufficient strength to break the emulsion and react with contaminations including lint, the treatment being conducted at a temperature above approximately 170° F. and preferably in the neighborhood of the boiling point of water, adding water to the mixture, agitating the mixture, and then separating renovated oil from the mixture.
11. The method of renovating contaminated, emulsified, car journal, lubricating oil which has been used with waste, which includes treating the oil by mixing therewith an alkaline solution of sufficient strength to break the emulsion and react with contaminations including lint, the treatment being conducted at a temperature above approximately 170° F. and preferably in the neighborhood of the boiling point of water, intermittently agitating the mixture, and separating renovated oil from the mixture.
12. The method of renovating contaminated, emulsified, car journal, lubricating oil which has been used with waste, which includes treating the oil by mixing therewith an alkaline solution of sufficient strength to break the emulsion and react with contaminations including lint, the treatment being conducted at a temperature above approximately 170° F. and preferably in the neighborhood of the boiling point of water, agitating the mixture, and separating renovated oil from the mixture.

- mately 170° F. and preferably in the neighborhood of the boiling point of water, intermittently agitating the mixture, mixing water therewith, and separating renovated oil from the mixture.
13. The method of renovating contaminated, emulsified, car journal, lubricating oil which has been used with waste, which includes treating the oil by mixing therewith an alkaline solution of sufficient strength to break the emulsion and react with contaminations including lint, the treatment being conducted at a temperature above approximately 170° F. and preferably in the neighborhood of the boiling point of water, agitating the mixture, mixing water therewith, again agitating, and separating renovated oil from the mixture.
14. The method of renovating contaminated, emulsified, car journal, lubricating oil which has been used with waste, which includes treating the oil by mixing therewith an alkaline solution of sufficient strength to break the emulsion and react with contaminations including lint, the treatment being conducted at a temperature above approximately 170° F. and preferably in the neighborhood of the boiling point of water, intermittently agitating the mixture, mixing water therewith, again agitating, and separating renovated oil from the mixture.
15. The method of renovating contaminated, emulsified, car journal, lubricating oil which has been used with waste, which includes treating the oil by mixing therewith an alkaline solution of sufficient strength to break the emulsion and react with contaminations including lint, the treatment being conducted at a temperature above approximately 170° F. and preferably in the neighborhood of the boiling point of water, agitating the mixture with air, and separating the renovated oil from the mixture.
16. The method of renovating contaminated, emulsified, car journal, lubricating oil which has been used with waste, which includes treating the oil by mixing therewith an alkaline solution of sufficient strength to break the emulsion and react with contaminations including lint, the treatment being conducted at a temperature above approximately 170° F. and preferably in the neighborhood of the boiling point of water, agitating the mixture with air, mixing water therewith, and separating the renovated oil from the mixture.
17. The method of renovating contaminated, emulsified, car journal, lubricating oil which has been used with waste, which includes treating the oil by mixing therewith an alkaline solution of sufficient strength to break the emulsion and react with contaminations including lint, the treatment being conducted at a temperature above approximately 170° F. and preferably in the neighborhood of the boiling point of water, and
- of the boiling point of water, intermittently agitating the mixture with air, and separating the renovated oil from the mixture.
18. The method of renovating contaminated, emulsified, car journal, lubricating oil which has been used with waste, which includes treating the oil by mixing therewith an alkaline solution of sufficient strength to break the emulsion and react with contaminations including lint, the treatment being conducted at a temperature above approximately 170° F. and preferably in the neighborhood of the boiling point of water, intermittently agitating the mixture with air, mixing water therewith, and separating the renovated oil from the mixture.
19. The method of renovating contaminated, emulsified, car journal, lubricating oil which has been used with waste, which includes treating the oil by mixing therewith an alkaline solution of sufficient strength to break the emulsion and react with contaminations including lint, the treatment being conducted at a temperature above approximately 170° F. and preferably in the neighborhood of the boiling point of water, intermittently agitating the mixture with air, mixing water therewith, again agitating with air, and separating the renovated oil from the mixture.
20. In a method of renovating journal box lubricating oil which has been used with waste, those steps which include dissolving a strong base caustic in water and mixing the solution with the oil before the temperature thereof has changed substantially from that produced by dissolving the caustic in the water.
21. In a method of renovating journal box lubricating oil which has been used with waste, those steps which include dissolving a strong base caustic in water and mixing the solution with the oil before the temperature thereof has changed substantially from that produced by dissolving the caustic in the water, the oil, at the time of mixing, being substantially at the same temperature.
22. The method of renovating contaminated, emulsified, car journal, lubricating oil which has been used with waste, which includes mixing the oil with an alkaline solution of sufficient strength to break the emulsion and react with contaminations including lint, and separating renovated oil from the mixture.
23. The method of renovating contaminated, emulsified, car journal, lubricating oil which has been used with waste, which includes treating the oil by mixing therewith an alkaline solution of sufficient strength to break the emulsion and react with contaminations including lint, the treatment being conducted at a temperature above approximately 170° F. and preferably in the neighborhood of the boiling point of water, and

separating renovated oil from the mixture.

24. The method of renovating contaminated, emulsified, car journal, lubricating oil which has been used with waste, which includes mixing the oil with an alkaline solution of sufficient strength to break the emulsion and react with contaminations including lint, intermittently agitating the mixture, and separating renovated oil from the mixture.

25. In a method of renovating contaminated, emulsified, car journal, lubricating oil which has been used with waste, those steps which include treating the oil by mixing therewith an alkaline solution of sufficient strength to break the emulsion and react with contaminations including lint, the treatment being conducted at a temperature above approximately 170° F. and preferably in the neighborhood of the boiling point of water, and cooling the mixture in the upper portion first.

26. In a method such as defined in claim 23, the step of permitting the temperature to drop somewhat below treating temperature before separating the oil from the mixture.

27. The method of renovating contaminated, emulsified, car journal, lubricating oil which has been used with waste, which includes mixing the oil with an alkaline solution of sufficient strength to break the emulsion and react with contaminations including lint, agitating the mixture, and separating renovated oil from the mixture.

28. The method of renovating contaminated, emulsified, car journal, lubricating oil which has been used with waste, which includes mixing the oil with an alkaline solution of sufficient strength to break the emulsion and react with contaminations including lint, agitating the mixture with air, and separating renovated oil from the mixture.

29. The method of renovating contaminated, emulsified, car journal, lubricating oil which has been used with waste, which includes mixing the oil with an alkaline solution of sufficient strength to break the emulsion and react with contaminations including lint, intermittently agitating the mixture with air, and separating renovated oil from the mixture.

30. In a method of renovating contaminated, emulsified, car journal, lubricating oil which has been used with waste, those steps which include mixing the oil with an alkaline solution of sufficient strength to break the emulsion and react with contaminations including lint, mixing water therewith, and separating renovated oil from the mixture.

31. The method of renovating contaminated, emulsified, car journal, lubricating oil which has been used with waste, which includes treating the oil by mixing therewith an alkaline solution of sufficient strength to break the emulsion and react with contaminations including

nations including lint, the treatment being conducted at a temperature above approximately 170° F. and preferably in the neighborhood of the boiling point of water, mixing water therewith, and separating renovated oil from the mixture.

32. In a method of renovating contaminated, emulsified, journal box lubricating oil which has been used with waste, the step which involves mixing the oil with an alkaline solution of strength sufficient to break the emulsion and react with contaminations including lint, the mixing being carried out with the solution and the oil at a temperature approximately between 170° F. and 200° F.

33. In a method of renovating emulsified, contaminated, journal box, lubricating oil which has been used with waste, those steps which include treating the oil by mixing therewith an alkaline solution of strength sufficient to break the emulsion and react with contaminations including lint, the treatment being conducted at a temperature above approximately 170° F. and preferably in the neighborhood of the boiling point of water, and mixing water therewith at a temperature approximately the same as that of the mixture being treated.

34. The method of renovating emulsified, contaminated, journal box, lubricating oil which has been used with waste, which includes mixing the oil with a strong base caustic solution, the caustic being from 3% to 6% of the oil by weight.

35. The method of renovating emulsified, contaminated, journal box, lubricating oil which has been used with waste, which includes mixing the oil with a strong base caustic solution, the caustic being from 20% to 25% of the solution by weight.

36. The method of renovating contaminated, emulsified, car journal lubricating oil which has been used with waste, which includes treating the oil by intimately contacting it with a solution of an alkali in water, the strength of which is sufficient to break the emulsion and react with contaminations including lint.

37. A lint-free journal box lubricating oil, reclaimed from contaminated journal box lubricating oil which has been used with waste.

38. The method of renovating contaminated, emulsified, car journal lubricating oil which has been used with waste, which includes treating the oil by intimately contacting it with a solution of an alkali in water, the strength of which is sufficient to break the emulsion and react with contaminations including lint, and adding water to the mixture.

39. The method of renovating contaminated, emulsified, car journal lubricating oil which has been used with waste, which in-

- cludes treating the oil by intimately contacting it with a solution of an alkali in water, the strength of which is sufficient to break the emulsion and react with contaminations including lint, the treatment being conducted at a temperature above approximately 170° F. and preferably in the neighborhood of the boiling point of water, and adding water to the mixture. 5 70
- 10 40. The method of renovating contaminated, emulsified, car journal lubricating oil which has been used with waste, which includes treating the oil by intimately contacting it with a solution of an alkali in water, the strength of which is sufficient to break the emulsion and react with contaminations including lint, adding water to the mixture, and agitating the mixture after the addition of water thereto. 15 80
- 20 41. The method of renovating contaminated, emulsified, car journal lubricating oil which has been used with waste, which includes treating the oil by intimately contacting it with a solution of an alkali in water, the strength of which is sufficient to break the emulsion and react with contaminations including lint, the treatment being conducted at a temperature above approximately 170° F. and preferably in the neighborhood of the boiling point of water, adding water to the mixture, and agitating the mixture after the addition of water thereto. 25 85
- 30 42. The method of renovating contaminated, emulsified, car journal lubricating oil which has been used with waste, which includes treating the oil by intimately contacting it with a solution of an alkali in water, the strength of which is sufficient to break the emulsion and react with contaminations including lint and intermittently agitating the mixture. 35 90
- 40 43. The method of renovating contaminated, emulsified, car journal lubricating oil which has been used with waste, which includes treating the oil by intimately contacting it with a solution of an alkali in water, the strength of which is sufficient to break the emulsion and react with contaminations including lint, the treatment being conducted at a temperature above approximately 170° F. and preferably in the neighborhood of the boiling point of water, and intermittently agitating the mixture. 45 95
- 50 44. The method of renovating contaminated, emulsified, car journal lubricating oil which has been used with waste, which includes treating the oil by intimately contacting it with a solution of an alkali in water, the strength of which is sufficient to break the emulsion and react with contaminations including lint, and agitating the mixture with air. 55 100
- 60 45. The method of renovating contaminated, emulsified, car journal lubricating oil which has been used with waste, which includes treating the oil by intimately contacting it with a solution of an alkali in water, the strength of which is sufficient to break the emulsion and react with contaminations including lint, the treatment being conducted at a temperature above approximately 170° F. and preferably in the neighborhood of the boiling point of water, and agitating the mixture with air. 65 105
- 70 46. The method of renovating contaminated, emulsified, car journal lubricating oil which has been used with waste, which includes treating the oil by intimately contacting it with a solution of an alkali in water, the strength of which is sufficient to break the emulsion and react with contaminations including lint, the treatment being conducted at a temperature above approximately 170° F. and preferably in the neighborhood of the boiling point of water and intermittently agitating the mixture with air. 75 110
- 80 47. The method of renovating contaminated, emulsified, car journal lubricating oil which has been used with waste, which includes treating the oil by intimately contacting it with a solution of caustic soda in water, the strength of which is sufficient to break the emulsion and react with contaminations including lint. 85 90
- 90 48. The method of renovating contaminated, emulsified, car journal lubricating oil which has been used with waste, which includes treating the oil by intimately contacting it with a solution of caustic soda in water, the strength of which is sufficient to break the emulsion and react with contaminations including lint, the treatment being conducted at a temperature above approximately 170° F. and preferably in the neighborhood of the boiling point of water. 95 100
- 100 49. The method of renovating contaminated, emulsified, car journal lubricating oil which has been used with waste, which includes treating the oil by intimately contacting it with a solution of caustic soda in water, the strength of which is sufficient to break the emulsion and react with contaminations including lint, and adding water to the mixture. 105 110
- 110 50. The method of renovating contaminated, emulsified, car journal lubricating oil which has been used with waste, which includes treating the oil by intimately contacting it with a solution of caustic soda in water, the strength of which is sufficient to break the emulsion and react with contaminations including lint, the treatment being conducted at a temperature above approximately 170° F. and preferably in the neighborhood of the boiling point of water, and adding water to the mixture. 115 120
- 120 51. As a new product, lint-free journal box lubricating oil, reclaimed from emulsified, contaminated, car journal lubricating oil which has been used with waste, by intimately 125 130

contacting the contaminated oil with a solution of an alkali in water the strength of which is sufficient to break the emulsion and react with contaminations including lint, and then separating the oil from the mixture.

5 In testimony whereof I have hereunto signed my name.

LEONARD D. GRISBAUM.

contacting the contaminated oil with a solution of an alkali in water the strength of which is sufficient to break the emulsion and react with contaminations including lint, and  
5 then separating the oil from the mixture.

In testimony whereof I have hereunto signed my name.

LEONARD D. GRISBAUM.

10

**CERTIFICATE OF CORRECTION.**

Patent No. 1,791,473.

Granted February 3, 1931, to

LEONARD D. GRISBAUM.

It is hereby certified that error appears in the printed specification of the above numbered patent requiring correction as follows: Page 6, strike out lines 2 and 3, comprising present claim 1, and insert the following claim 1:

1. The method of renovating contaminated, emulsified, car journal lubricating oil which has been used with waste, which includes treating the oil by intimately contacting it with a solution of an alkali in water, the strength of which is sufficient to break the emulsion and react with contaminations including lint, the treatment being conducted at a temperature above approximately 170°F. and preferably in the neighborhood of the boiling point of water.;

and that the said Letters Patent should be read with this correction therein that the same may conform to the record of the case in the Patent Office.

Signed and sealed this 3rd day of March, A. D. 1931.

(Seal)

M. J. Moore,  
Acting Commissioner of Patents.

50

55

60

65

CERTIFICATE OF CORRECTION.

Patent No. 1,791,473.

Granted February 3, 1931, to

LEONARD D. GRISBAUM.

It is hereby certified that error appears in the printed specification of the above numbered patent requiring correction as follows: Page 6, strike out lines 2 and 3, comprising present claim 1, and insert the following claim 1:

1. The method of renovating contaminated, emulsified, car journal lubricating oil which has been used with waste, which includes treating the oil by intimately contacting it with a solution of an alkali in water, the strength of which is sufficient to break the emulsion and react with contaminations including lint, the treatment being conducted at a temperature above approximately 170°F. and preferably in the neighborhood of the boiling point of water.;

and that the said Letters Patent should be read with this correction therein that the same may conform to the record of the case in the Patent Office.

Signed and sealed this 3rd day of March, A. D. 1931.

(Seal)

M. J. Moore,  
Acting Commissioner of Patents.